

## UNITED STATES PATENT OFFICE

2,063,337

PROCESS OF FINISHING LEATHERS AND  
PRODUCTJames T. Power, Wilmington, Del., assignor to  
Atlas Powder Company, Wilmington, Del., a  
corporation of DelawareNo Drawing. Application January 31, 1935,  
Serial No. 4,308. Renewed May 14, 1936

20 Claims. (Cl. 149—6)

This invention relates to the finishing of leathers and particularly to the finishing of soft or light leathers. The invention has for its object to improve the finish of leathers. These 5 improvements consist of (1) the production of a softer and more flexible finished leather than is obtained with present known materials or methods; (2) a reduced susceptibility to changes in the properties of leathers with changes in humidity conditions. Further objects and advantages will be set forth in the following description and in the claims appended thereto.

The animal skins from which leather is made consist of a natural fabric of interwoven fibers. 15 The leather tanner cannot alter the fabric structure to any appreciable extent, and so his problem is the treatment and finishing of the fiber structure given him, so as to produce the desired texture. The skin must first be freed from dirt 20 and blood and other adventitious material, and the hair, epidermis and flesh removed. Then the skin must be so treated as to reduce its sensitiveness to water and render it resistant to putrefaction. This in turn must be followed by 25 a series of finishing operations designed to give the skin the proper mechanical feel, surface appearance and waterproof or water-resisting characteristics.

The types of tanning and finishing operations 30 obviously depend on the final use of the leather, e. g. heavy leather for sole leather, etc., and light or soft leather for shoes, gloves and the like. Thus the various steps in preparing a glacé kid leather, for example, would probably 35 include soaking, painting, liming and deliming, puering, pickling, chrome tanning, washing and neutralizing, dyeing, fatliquoring, damping and staking, oiling off or clearing and seasoning, glazing and the final finishing. These steps may be 40 modified in a number of ways by those skilled in the art in order to produce various effects or finishes. For example, an enzyme treatment may be substituted for or used in addition to the steps of painting, liming and deliming.

45 This invention is mainly concerned with the treatment of the skin following its conversion to leather by the tanning operation. For example, with a chrome tanned leather, if it be dried out, it will be converted into horn by the adhesion of the fibers of the mass due to the plasticity of their surfaces, and it cannot be wet back to its former soft hydrated state. It is 50 therefore imperative to fatliquor tanned leather after tanning and before drying out, so as to prevent the coalescence of the fibers on dehydra-

tion. Once thus properly dried, the fibers have lost their plasticity and the leather can be wet back indefinitely without adhesion of the fibers.

It has been the practice to fatten with glycerine mixed with vegetable or other oils; glycerine and soaps of these oils; glycerine and sulphonated oils; egg yolk and oils; or egg yolk alone. Various combinations of the above are sometimes used depending upon the particular hides undergoing treatment and the finish desired. Glycerine when thus used depends in part 10 for its effect upon its hygroscopic and softening nature which causes the retention of moisture in the fabric; thus enhancing the fullness and softening effect.

Glycerine as a finishing agent is at a disadvantage because of its extreme avidity for moisture under conditions of high humidity. Leathers treated with glycerine as a finishing agent when exposed to high humidity show a large 15 increase in surface area, which is a disadvantage; for example, in the manufacture of leather for use in making shoes and similar articles where increase in surface area should be at a minimum under conditions of high humidity. Leathers 20 containing any considerable amount of glycerine absorb so much moisture when exposed to conditions of high humidity that they become limp, exhibiting what is known to the art as a "raggy" 25 effect. Consequently the tanners or finishers of leather cannot take full advantage of the softening 30 effect of glycerine, being forced to keep the glycerine concentration in the finishing operations low enough to avoid the difficulty mentioned above.

Now I have found that some of the hexahydric alcohols as well as many water soluble derivatives of hexahydric alcohols offer distinct advantages as ingredients in the finishing process. An example of a hexahydric alcohol which is 35 suitable for use in the finishing process is sorbitol. In the finishing process with equal concentrations, sorbitol produces a greater softening effect upon leathers than does glycerine. Sorbitol is a hygroscopic substance, but I find that 40 while sorbitol absorbs approximately the same amount of moisture from atmospheres of low humidities as does glycerine, at high relative humidities it absorbs much less moisture than does glycerine. The increase in area of leather 45 finished with sorbitol when exposed to high humidity conditions is much less than in the case of leathers treated with glycerine.

The amounts of moisture absorbed by glycerine and sorbitol when allowed to come to equilibrium 50

with atmospheres of various relative humidities are shown in the following table:

| Relative humidity | Weight of moisture absorbed by 100 g. of |               |
|-------------------|------------------------------------------|---------------|
|                   | Glycerine (g.)                           | Sorbitol (g.) |
| Percent           |                                          |               |
| 20                | 5.8                                      | 4.2           |
| 40                | 17.8                                     | 13.7          |
| 80                | 108                                      | 61.0          |

Another hexahydric alcohol which is hygroscopic and may be used in place of glycerine in finishing leather is iditol.

Among the water soluble hygroscopic derivatives of hexahydric alcohols I may mention mono-anhydro sorbitol or sorbitan, dianhydro sorbitol or sorbide, monoanhydro mannitol or mannitan, dianhydro mannitol or mannide, monoanhydro dulcitol or dulcitan and dianhydro dulcitol or dulcide.

The leather treated with these compounds will show smaller variations in moisture content, when subjected to varying humidity conditions, than will the same leather treated with glycerine. Thus the finisher can take full advantage of the superior softening action of sorbitol, for example, without fear of the development of "ragginess" and possible stretching should the leather be exposed to atmospheres of high humidity.

Moreover, I have found that a leather treated with a hygroscopic hexahydric alcohol, or a water soluble hygroscopic anhydro derivative of a hexahydric alcohol at the proper stage of the finishing operation, has a superior "body" to that of a similar leather treated with a like concentration of glycerine.

In the following examples I have chosen as the preferred embodiment of my invention the hexahydric alcohol sorbitol. However, it is to be understood that proper amounts of iditol, sorbitan, sorbide, etc., may be substituted for the sorbitol if so desired.

The following example represents one recipe for fat liquor to follow the tanning operation:

|                    |      |       |
|--------------------|------|-------|
| I. Castor oil soap | lbs. | 3     |
| Sorbitol           | lbs. | 2     |
| Castor oil         | lbs. | 1 1/2 |
| Boiling water      | lbs. | 10    |

Other vegetable oils, sulphonated oils, animal and marine oils may be used in place of castor oil, as for example:

|                 |      |       |
|-----------------|------|-------|
| II. Sorbitol    | lb.  | 1     |
| Castile soap    | lbs. | 1 1/2 |
| Neat's-foot oil | lbs. | 2     |
| Borax           | oz.  | 4     |
| Water           | lbs. | 150   |

Another example of a fat liquor suitable for treating the leather after tanning is as follows:

|                 |       |       |
|-----------------|-------|-------|
| III. Degas      | lbs.  | 10    |
| Olive oil       | lbs.  | 10    |
| Sorbitol        | lbs.  | 4     |
| Soft soap       | lbs.  | 5     |
| Water at 140° F | gals. | 60-70 |

The skins are tumbled in this emulsion for a period in the neighborhood of 45 minutes and are then hung on a trestle for about 30 minutes to let the fat penetrate the leather.

However, the sorbitol treatment may occur in the oiling off operation, in which case it may or

may not have been used in the fat liquor. This must be determined by individual practice. The leather may be treated as follows:

|                                            |      |   |
|--------------------------------------------|------|---|
| IV. Sorbitol syrup of 85% sorbitol content | lb.  | 1 |
| Water                                      | lbs. | 3 |

I have found that a superior result was obtained with this sorbitol recipe in comparison with a mixture of 1 part of C. P. glycerine and 1 part water. The sorbitol mixture given in Example IV can be applied by spreading the tanned, colored and fat liquored skin on a flat surface with the grained side up. The skin is then lightly brushed manually or by machine with a brush dipped in the sorbitol mixture. Immediately after the sorbitol treatment the skins are hung up to dry. Sometimes the tanner prefers to give the skins a light coating of neat's-foot oil applied on the grain side of the skin following the sorbitol treatment and before drying.

Other ingredients may be added to the sorbitol solution, such as blood or egg albumen, milk, casein and dyes such as nigrosine, logwood extract and hematine. Such a finish is made up as follows:

|                  |          |
|------------------|----------|
| V. Blood albumen | 15%      |
| Nigrosine        | 1%       |
| Sorbitol syrup   | 1/2%     |
| Milk             | 10%      |
| Water            | 73 1/2 % |

It is, moreover, possible, after the leather has been dyed, by rubbing sorbitol in on the non-dyed side to give it the necessary degree of suppleness.

A gloss can then be developed by glazing and the final finishing for the particular use follows.

While I have described the invention somewhat specifically for the purpose of establishing a clear disclosure so as to enable those skilled in the art to appreciate the value of this invention, it is understood that I am not to be limited to such specific disclosure, but that we include within its scope such changes in practice as fairly fall within either the terms or spirit of the appended claims.

While I have disclosed the hygroscopic hexahydric alcohols and the water soluble, hygroscopic, anhydro derivatives of hexahydric alcohols as advantageous in finishing leathers it is to be understood that solutions of these substances may be applied. Also instead of the pure substances I have used the technical products containing relatively small amounts of ash, sugar and other organic impurities, and the results obtained with the technical products were equally as good as those obtained with the pure substances.

Having described my invention, what I claim is:

1. A process of finishing leather which comprises treating the leather with a compound selected from the group consisting of the hygroscopic hexahydric alcohols and the water soluble, hygroscopic, anhydro derivatives of the hexahydric alcohols.

2. A process of finishing leather which comprises treating the leather with a hygroscopic hexahydric alcohol.

3. A process of finishing leather which comprises treating the leather with sorbitol.

4. A process of finishing leather which comprises treating the leather with iditol.

5. A process of finishing leather which comprises treating the leather with a water soluble,

hygroscopic, anhydro derivative of a hexahydric alcohol.

6. A process of finishing leather which comprises treating the leather with sorbitan.

7. A process of finishing leather which comprises treating the leather with a mixture containing an oil and a compound selected from the group consisting of the hygroscopic hexahydric alcohols and the water soluble, hygroscopic, anhydro derivatives of the hexahydric alcohols.

8. A process of finishing leather which comprises treating the leather with a mixture containing a hygroscopic hexahydric alcohol and an oil.

9. A process of finishing leather which comprises treating the leather with a mixture containing sorbitol and an oil.

10. A process of finishing leather which comprises treating the leather with a mixture containing an oil, a soap, and a compound selected from the group consisting of the hygroscopic hexahydric alcohols and the water soluble, hygroscopic, anhydro derivatives of the hexahydric alcohols.

11. A process of finishing leather which comprises treating the leather with a mixture containing a hygroscopic hexahydric alcohol, an oil, and a soap.

12. A process of finishing leather which comprises treating the leather with a mixture containing sorbitol, an oil, and a soap.

13. In the process of finishing leather the step of fat liquoring which comprises treating the leather with sorbitol.

14. A fat liquor bath for finishing leather, said bath containing sorbitol and an oil.

15. In the process of finishing leather the step of oiling off which comprises treating the leather with sorbitol.

16. An article of manufacture comprising leather and a compound selected from the group consisting of the hygroscopic hexahydric alcohols and the water soluble, hygroscopic, anhydro derivatives of the hexahydric alcohols.

17. An article of manufacture comprising leather and a hygroscopic hexahydric alcohol.

18. An article of manufacture comprising leather and sorbitol.

19. An article of manufacture comprising leather and a water soluble, hygroscopic, anhydro derivative of a hexahydric alcohol.

20. An article of manufacture comprising leather and sorbitan.

JAMES T. POWER.

15

20

25